

## UNITED STATES PATENT OFFICE

1,975,120

## ALLOY

Roy E. Paine, Cleveland, Ohio, assignor, by  
mesne assignments, to Magnesium Develop-  
ment Corporation, a corporation of Delaware

No Drawing. Application January 4, 1934,  
Serial No. 705,285

## 2 Claims. (Cl. 75—1)

The invention relates to magnesium base al-  
loys. An object of the invention is the develop-  
ment of alloys of this nature containing tin and  
cobalt.

I have discovered that when cobalt is added to  
5 magnesium base alloys containing tin, the re-  
sulting alloys undergo an improvement in both  
tensile strength and elongation. I have also dis-  
covered that the magnesium-tin-cobalt alloys  
10 may be further improved by suitable thermal  
treatments.

As an illustration of the effect produced by the  
addition of cobalt to a magnesium base alloy, I  
have made up an alloy of this nature containing  
5.0 per cent of tin, the balance being commercial  
15 magnesium. This alloy had a tensile strength,  
in the cast condition, of 18,380 pounds per square  
inch and an elongation of 5.0 per cent in two  
inches. A second alloy containing, in addition  
20 to 5.0 per cent of tin, 0.5 per cent of cobalt  
had in the cast condition a tensile strength of  
18,940 pounds per square inch and an elongation  
of 5.7 per cent in two inches. A third alloy  
25 containing 2.0 per cent of cobalt, in addition to  
5.0 per cent of tin, had in the cast condition  
a tensile strength of 20,920 pounds per square  
inch and an elongation of 6.3 per cent in two  
inches. It may be observed that the above addi-  
30 tions of cobalt have successively increased both  
strength and elongation.

30 A thermal treatment of 19 hours at 525° centi-  
grade followed by quenching increased the  
strength of the 0.5 per cent cobalt alloy from  
18,940 pounds to 23,680 pounds per square inch  
35 and the elongation from 5.7 per cent to 8.8 per  
cent in two inches. After the same thermal treat-  
ment the tensile strength of the 2.0 per cent cobalt  
alloy increased from 20,920 pounds to 24,670  
40 pounds per square inch and the elongation in-  
creased from 6.3 per cent to 9.2 per cent in two  
inches.

Another magnesium-tin alloy containing 10.0  
per cent of tin, the balance being commercial  
magnesium, was made up to contain, in addition,  
45 1.0 per cent of cobalt. This alloy on being heated

for 19 hours at 525° centigrade and quenched  
had a tensile strength of 23,220 pounds per square  
inch and an elongation of 7.8 per cent in two  
inches. After an additional "aging" treatment  
50 of 20 hours at 150° centigrade the tensile strength  
increased to 26,750 pounds per square inch and  
the elongation to 9.8 per cent in two inches. In  
alloys of the type herein discussed the cobalt  
may be present in amount between about 0.1  
55 per cent and 4.0 per cent and may be added to  
magnesium-tin alloys containing from about 0.1  
per cent to about 20.0 per cent of tin. As a pre-  
ferred composition I have used an alloy contain-  
ing 5.0 per cent of tin and 1.0 per cent of cobalt,  
60 the balance being commercial magnesium.

The alloys are susceptible to variations in their  
physical properties by thermal treatments at tem-  
peratures most effective between about 425° and  
525° centigrade and may be given additional  
"aging" treatments between about 100° and 200°  
75 centigrade. They may be compounded in any  
of the ways familiar to the art, such as by adding  
to the molten magnesium bath the alloying ele-  
ment when its melting point is below that of the  
magnesium, or approximates it, or by adding the  
80 alloying element in the form of a magnesium-  
rich alloy or "hardener" when its melting point  
considerably exceeds that of the magnesium.

The alloys disclosed herein may be extruded  
over the whole range disclosed, and may be  
85 forged or otherwise mechanically deformed when  
the amount of added alloying elements does not  
become too great a proportion of the whole.

In this specification and the appended claims  
the term "magnesium base alloy" signifies an al-  
loy containing more than 50 per cent magnesium.

## I claim:

1. A magnesium base alloy containing from 0.1  
per cent to 20.0 per cent of tin and from 0.1 per  
cent to 4.0 per cent of cobalt, the balance being  
85 substantially all magnesium.

2. A magnesium base alloy containing about  
5.0 per cent of tin and 1.0 per cent of cobalt, the  
balance being substantially all magnesium.

ROY E. PAYNE.